

E. E. WATTS.  
PROCESS OF EXTRACTING ZINC FROM ITS ORES OR COMPOUNDS.  
APPLICATION FILED NOV. 20, 1913.

1,111,201.

Patented Sept. 22, 1914.



Inventor

E. E. WATTS.

Witnessed

Edwin B. Hunt.

Edwin B. Hunt

By A. B. Gleeson & Co.

Attorneys

# UNITED STATES PATENT OFFICE.

ERNEST ESTRAM WATTS, OF KINGSTON, ONTARIO, CANADA.

## PROCESS OF EXTRACTING ZINC FROM ITS ORES OR COMPOUNDS.

1,111,201.

Specification of Letters Patent. Patented Sept. 22, 1914.

Application filed November 20, 1913. Serial No. 802,128.

To all whom it may concern:

Be it known that I, ERNEST ESTRAM WATTS, a subject of the King of England, residing at Kingston, in the Province of 5 Ontario and Dominion of Canada, have invented certain new and useful Improvements in Processes of Extracting Zinc from its Ores or Compounds; and I do declare the following to be a full, clear, and exact description 10 of the invention, such as will enable others skilled in the art to which it appertains to make and use the same.

This invention relates to a process for extracting zinc from its ores.

15 The object of the invention is to obtain zinc from ores or compounds containing it in a cheap and convenient manner which is especially adapted for use in certain localities.

20 In the accompanying drawings are shown one form of apparatus used in connection with this improved process, Figure 1 representing a plan view thereof; Fig. 2 an end elevation partly in section; and Fig. 3 a side 25 elevation partly in section.

In the standard method of extracting zinc from ores or compounds by distillation, the most skilful attention is necessary, and then losses of up to 25 per cent. of the metal occur. There is also considerable wear and tear upon the retorts and furnaces. Moreover, zinc ores or products lower than 40 per cent. in zinc cannot usually be treated at a profit by this method. For these reasons, 30 zinc mines in localities situated at a distance from fuel supplies and suitable clays for retort manufacture are unable to profitably produce zinc. Furthermore, for the following reasons, the recovery of zinc by 35 electrolytic methods has hitherto been but slightly successful, (1) the power consumption necessary to deposit a strongly electro-positive metal like zinc from aqueous solution by using insoluble anodes, is high; (2)

40 great difficulty has been experienced in obtaining a good cathodic deposit of zinc; (3) great difficulty has been experienced in obtaining an electrolyte of the necessary constant composition and purity. By my in-

45 vention, I have overcome most of these disadvantages, and very largely corrected the others and I propose to produce a compound or product high in zinc and to then introduce this compound or product in the form 50 of a paste into an electrolytic bath of a

nearly saturated solution of a zinc salt in anode compartments of the said bath. Upon the passage of a suitable current zinc will deposit upon the cathodes, and the acid liberated by the electrolysis will be constantly 60 used up in dissolving zinc from the compound or product in the anode compartments in the form in which it already exists in the bath. The concentration and composition of the electrolyte will thus be maintained constantly at the conditions for high current efficiency and good cathode deposit. By the aid of efficient circulation, and the addition of certain substances which I shall 65 later specify, high current efficiency may be further assured and the character of the deposit improved. The various steps in this system of zinc extraction are later more particularly described.

In the form of apparatus herein shown a 75 plurality of tanks 1, 2 and 3 are shown arranged in series with circulation pipes as 4 connecting the adjacent tanks, the circulation taking place by gravity as each tank is disposed slightly lower than its predecessor in the series. Cathodes 5 are shown extending transversely of each tank with anodes 6 alternating therewith. Each of the anodes is shown disposed in a compartment 7 which compartments are composed 80 of any suitable material which will allow the passage of the liquid of the bath therethrough, but will prevent the passage of the paste disposed therein as will be hereinafter described. The points of contact between 85 the anodes and cathodes are shown at 8 and 9 respectively which are herein shown in the form of lugs or projections at the tops of the plates forming the anodes and cathodes, these lugs being shown in Fig. 2 as projecting over the side of the tank and holding the plates suspended. Contact between the plates and the tank is prevented by insulation between the legs and the walls of the tank except at the points indicated. The 90 stipple shown at 10 in the compartments 7 represent the paste which is employed in the process as will be hereinafter described.

95 Any suitable method may be employed to obtain the compounds or products high in zinc for introduction into the electrolytic bath, several instances are given below, to wit: From zinc ores amenable to concentration, I may concentrate by ore-dressing methods suited to the particular ore and so 100 105 110

obtain a concentrate or product high in zinc. This concentrate must then be roasted until practically free from sulfur as sulfid and sulfate of zinc and then introduced 5 into the bath in the manner to be described. Zinc products or by-products not amenable to concentration, such as blue powder, or impure zinc oxid, free from objectionable impurities that would tend to foul the bath, 10 such as sulfids and sulfites, are suitable products for introduction into the bath. In case of the presence of objectionable impurities, it will be necessary to free the product from these if possible before charging to the bath. 15 Complex lead zinc ores may be treated in the following manner to obtain a compound or product suitable for charging to the bath, to wit: First the ore is roasted if found necessary and then the zinc contents in the form 20 of oxid volatilized in any suitable manner from the roasted or unroasted ore.

A further method of treating complex lead zinc ores high in sulfur in order to obtain a compound or product suitable for charging 25 to the electrolytic bath, is as follows: The ore is first finely crushed, roasted in an oxidizing atmosphere, and the roast leached with sulfurous acid. The zinc dissolves as zinc bisulfite, and from the solution I precipitate the zinc as zinc monosulfite by expelling the sulfur dioxide from the solution by boiling. I then remove the zinc monosulfite precipitate and roast it to remove all 30 combined and uncombined sulfur, so producing an impure zinc oxid product suitable for charging to the electrolytic bath.

It is known that zinc sulfate forms in roasting blende. This is dissolved upon leaching with sulfurous acid and cannot be 40 precipitated by boiling. I have also found that if the roasting is performed at a temperature at about 750° C. or below, that in addition to some zinc sulfate, some iron sulfate also remains undecomposed, and, upon 45 leaching and attempting to precipitate the zinc by boiling, up to 50% of the zinc in solution will not precipitate but remains in solution of sulfate. It is also known that in roasting blende at a temperature exceeding 50 950° C., that zinc and iron are liable to combine to form a compound known as zinc ferrite which is insoluble in sulfurous acid. I avoid these difficulties by carrying on the roasting operation at a temperature of about 55 700° C. to 800° C. until the sulfur is largely removed and then at a temperature of about 900° C. to 950° C. until the roast is completely finished. Then, the zinc and iron sulfates are practically completely decomposed, and but little zinc ferrite is formed. I find that the roasts that are finished at a 60 high temperature are difficult to extract by means of sulfurous acid for there appears to be an insoluble film inclosing the grains of 65 the roast. This difficulty I overcome by re-

grinding the roast to a fine powder. This finely pulverized roast I then leach with sulfurous acid in a suitable apparatus in which the sulfur dioxide of the roaster gases is dissolved in water under slight pressure. I 70 also propose utilizing the sulfur dioxide gas generated by the precipitation of the solution and by the roasting of the precipitate in the same or a similar apparatus. The zinc from the roast goes into solution in sulfurous 75 acid as zinc bisulfite. Lime present in the ore will also go into solution.

The ratio of solution to ore varies with the amount of zinc in the ore, and in general the more concentrated the solution the greater 80 is the ease with which the zinc is precipitated from it. (With a thirty per cent. zinc ore I have obtained excellent results using six parts of solution to one of ore.)

Having obtained the zinc in solution, the residue, containing most of the lead, iron, and precious metals of the original ore, is separated from the solution by decantation, or filtration, or both. Having precipitated the zinc monosulfite, I propose to first cool the solution, and remove the precipitate by decantation and filtration, for I have found that, if the solution is not first cooled, the zinc monosulfite will crystallize out of the solution into the pores of the 95 filtering medium and so stop the operation. The precipitate obtained in this manner I propose to roast at a temperature between 800° C. and 1000° C. in an oxidizing atmosphere. As the precipitate roasts very 100 readily I have found that in about two hours, without the addition of any other substances, that I can obtain a product practically free from combined or uncombined sulfur, and thus a product suitable 105 for charging to the electrolytic tanks. The solution from the precipitation of the zinc monosulfite will contain some iron which will settle out from the solution after standing twenty-four hours. The clear solution can then be decanted off. Zinc sulfate will gradually accumulate in these solutions as they are used and re-used and these solutions may be freed from zinc, and the zinc recovered, by treating the solutions with 110 some cheap precipitant such as soda ash or lime.

Having obtained products or compounds of zinc suitable for charging to the electrolytic tanks, these compounds or products 115 are mixed to a thin paste with a solution of zinc sulfate and the paste charged to the electrolytic tanks, and treated in a manner to be described. It has been found that if the products or compounds are charged 120 to the tanks without mixing them to a thin paste, they will cake, and consequently the zinc is thoroughly extracted from the exterior only of the cake. The compounds or products are charged to the bath to the 125 130

compartments 7 at the anodes after mixing them to a thin paste with a solution of zinc sulfate. These compartments are simply portions of the tank surrounding the 5 anodes partitioned off by any suitable material which will allow the passage of the liquid of the bath, but prevent the passage of the paste from the compartments. Thus the bath is kept free from solids and 10 constantly at the composition and concentration necessary for high current efficiency and good cathode deposit.

It is known, that in the electrolysis of a solution of zinc sulfate, that zinc is deposited at the cathode, and sulfuric acid 15 generated at the anode by secondary reaction. If this acid is not removed in some manner, after the acid in the bath reaches a certain low concentration, hydrogen and 20 not zinc is liberated at the cathode. Thus, by this method of introduction of a compound or product containing zinc at the anode, the acid is immediately consumed and the concentration of the solution with 25 respect to zinc kept constant. At the anodes, zinc appears to go into solution largely to the exclusion of the iron, which goes into solution but to a limited extent, and does not interfere with the obtaining 30 of a pure zinc deposit. Thus, a nearly saturated solution of the sulfate of a strongly electro-positive metal like zinc can maintain itself comparatively pure in the presence of less electro-positive metals such as iron. 35 Thus, in the system of zinc extraction, I obtain high current efficiency and good cathode deposits, and maintain the solution constantly at the concentration and composition necessary for obtaining these. As 40 the depleted residue in the anode compartments is removed, fresh material is added, and the process is thus continuous. The residue is separated from the solution, and the solution returned to the tanks.

45 During the process there is some loss of solution due to evaporation and losses in handling. This loss may be corrected by the addition of fresh solution, or by maintaining the volume of the solution constant 50 by the addition of water, and adding the necessary amount of zinc sulfate. This zinc sulfate may be obtained by controlling the conditions during the roasting of the various zinc and sulfur holding products, or, 55 may be obtained by exposing the zinc monosulfite precipitate from the sulfurous acid leach to the atmosphere for a few weeks. The zinc monosulfite is then practically completely oxidized to sulfate and this zinc sulfate may be charged to the bath. It is of 60 course inadvisable to have large quantities of zinc sulfate added to the bath in the usual addition of the pastes, and I preferably add just sufficient zinc sulfate, to make up for 65 unavoidable losses. If large amounts of

zinc sulfate were added in the pastes, the acid generated through electrolysis could not be neutralized in the manner above described.

In the anode compartments insoluble 70 anodes of lead are used and these in time become coated with an insoluble coating of oxid of lead, iron and manganese. For cathodes, stationary sheets of zinc, copper or iron are preferably employed. 75

For the electrolytic bath, a solution of zinc sulfate kept constantly at a concentration of twelve per cent. or over of zinc in the manner above described, is preferably used, but a zinc chlorid solution may be 80 used if desired. I have found that the presence of such substances as gelatin, glue, starch, or sugar, in the bath improve the character of the zinc deposit tending to make it more dense and compact. 85

In this system of zinc extraction, the electrolytic tanks shown at 1, 2 and 3 are preferably arranged in series with the electrodes in each tank in parallel, and one or two tanks in the series preferably having no current passing therethrough, but in which the anode compartments thereof remain charged. Thus, the solution during circulation has additional opportunity to come in contact with the contents of the anode compartments, and, at any time, any tank may be thrown out of the circuit for purposes of cleaning, repairing or removing the cathodes, without interfering with the rest of the circuit, the extra tank being substituted. 95 100

During the electrolysis I find that I can obtain good results with current densities at the cathodes of from 2 amps. per sq. dm. to 5 amps. per sq. dm., or 18 amps. per sq. ft. 105 to 45 amps. per sq. ft., and under good conditions, the voltage corresponding to these current densities will vary from 3.5 volts to six volts, and a current density of about 2.5 amps. per sq. dm. should be maintained with 110 a difference of potential of 3.5 volts between electrodes.

The action of sulfurous acid upon oxid of zinc is well known, as is also the possibility of the electro-deposition of zinc from a zinc 115 sulfate or zinc chlorid solution, but, the combination and modifications of these processes I claim as my invention.

What I claim as new is:

1. A process of extracting zinc which 120 comprises mixing a material containing a high percentage of zinc in a non-elemental condition with a solution of zinc sulfate relatively free from dissolved iron compounds, in proportions to form a thin paste, charging said paste into the anode compartment of an electrolytic cell containing an electrolyte consisting of a highly concentrated solution of zinc sulfate, said solution being relatively free from iron compounds, and then 125 130

passing a suitable electric current through said cell, whereby the zinc is deposited at the cathodes.

2. A process of extracting zinc electrolytically which comprises first mixing a product high in zinc existing in a non-elemental condition with a sufficient quantity of a solution of a zinc salt to form a paste, said solution being substantially free from iron, charging said paste into the anode compartment of an electrolytic cell containing an electrolyte consisting of a substantially non-ferruginous solution of a zinc salt, passing an electric current through said cell, and thereby depositing metallic zinc at the cathode, the material surrounding the anode being kept separate from the liquid surrounding the cathode.

3. A process of extracting zinc electrolytically which comprises mixing impure zinc oxide substantially free from elemental zinc with a sufficient amount of a solution of zinc sulfate to form a paste, said solution of zinc sulfate being relatively free from dissolved iron compounds, introducing said paste into the anode compartment of an elec-

trolytic cell, containing an electrolyte comprising a solution of zinc sulfate, passing a current of electricity through said cell, thereby depositing metallic zinc at the 30 cathode.

4. A process of separating metallic zinc, which comprises mixing a material containing zinc in a non-elemental condition with a sufficient amount of a solution of zinc sulfate to form thin paste, introducing said paste into the anode compartments of an electrolytic cell containing an electrolyte consisting of a solution of zinc sulfate, containing about 12% of zinc, said electrolyte 40 also containing an organic material capable of rendering the zinc deposit dense and compact, and passing a suitable electric current through said cell, whereby zinc is deposited, at the cathodes.

In testimony whereof I have hereunto set my hand in presence of two subscribing witnesses.

ERNEST ESTRAM WATTS.

Witnesses:

GEO. H. SMYTHE,  
ANNA E. HANLON.